

May 16, 1939.

M. D. CURRAN

2,158,816

COKE MAKING PROCESS

Filed April 2, 1937

Fig. 1.



Fig. 2.

Inventor:

Maurice D. Curran

By

Wilkinson, Huxley, Bryant & Wright  
Attorneys.

## UNITED STATES PATENT OFFICE

2,158,816

## COKE MAKING PROCESS

Maurice D. Curran, Glendale, Mo., assignor to  
 Tar & Petroleum Process Company, Chicago,  
 Ill., a corporation of Illinois

Application April 2, 1937, Serial No. 134,552

10 Claims. (Cl. 202—9)

The present invention relates to improvements in coke making processes.

The present application is in part a continuation of application Serial No. 91,325, filed July 18, 1936, by the present applicant. Subject matter analogous in some respects to the subject matter of this application is described and claimed in applicant's co-pending application Serial No. 117,032.

10 More particularly the present invention relates to improved processes for controlling the characteristics of the coke resulting from the treatment of coal or other hydrocarbon containing material. The invention has particular applicability to 15 methods of manufacturing coke in which the layer of coal or equivalent material is shallow relative to the width thereof. Stated more particularly, the present invention relates to methods of manufacturing coke employing coke ovens of the 20 Knowles type, an example of which is illustrated and described in the patent to Knowles and McIntyre No. 1,635,280, patented July 12, 1927. According to the type of oven referred to, coal or equivalent material is disposed on a horizontal 25 floor heated by flues extending beneath said floor, the coking floor forming a part of the coking chamber, the oven having means for charging coal, means for withdrawing vapors and gases, means for sealing the ends of the chamber, and 30 means permitting the pushing of the resulting coke out of the coking chamber.

The coking process as carried out in the Knowles type of oven differs materially from the coking process as carried on in ordinary by- 35 product ovens in which the vertical height of the coal charge is great relative to the width thereof. In the ovens just referred to the vapors of distillation, together with the water vapor resulting from the drying of the coal, proceed upward and outward through the mass of coke lying adjacent to the coking walls. Except at the top of the coking charge, practically no vapors or gases pass through the coal mass in the middle of the oven, since the resistance of the latter to 40 fluid flow is greater than the resistance through the coke and upward along the side walls. The consequence is that the heat necessary for coking is supplied to the coal by conduction rather than by convection, and the coking zone is very 45 narrow, not over a fraction of an inch in thickness. By "coking zone" is meant the narrow and progressively moving body of liquid coal which results from the application of heat and which contains the hydrocarbons subsequently given off, leaving the coke. This condition of the cok-

ing zone is due to the fact that the heat is not carried inward to the mass of coal by the passage of hot vapors or gases.

According to the method of coking in which the bed of coal or its equivalent is shallow in 5 comparison to its width and in which the heat is applied below the bed of coal or the like, vapors of distillation, water vapors and fixed gases from the coal adjacent to the bottom of said bed are liberated at the beginning of the coking period, a substantial portion of these vapors and 10 gases passing upward through the coal and imparting their heat to the cooler coal mass. This results, first, in the vaporization of water in the coal and then in vaporization of volatile matters 15 and subsequent partial condensation of the vapors, provided the temperature in the upper portion of the charge is sufficiently low, followed by redistillation and elimination from the coal mass as the coking process proceeds. The passage of 20 vapors and gases through the coal mass results in a transfer of heat by means of convection to the coal mass and an increased thickness of the coking zone which may attain a thickness of two 25 inches or more in the case of coals having a high coking index. The result of this additional thickness in the coking zone is a trapping of vapors or gases within the coking zone and the forming of bubbles by said vapors and gases. The resistance of the thickened coking zone leads 30 to an unusually porous structure in the coke which in turn increases the reactivity of the coke to oxygen, and, other things being equal, increases combustibility.

An object of the present invention is to provide 35 an inexpensive process for making a low volatile coal suitable for blending with a high volatile coal for the manufacture of coke.

A further object is to provide a process of making the low volatile coal above referred to from 40 the same kind of coal with which it is to be mixed later in the manufacture of coke.

A further object is to provide the low volatile coal referred to at the same time that the mixture is being coked without requiring additional 45 apparatus or additional processes.

A further object is to provide an improved method for producing a commercially desirable coke without the necessity for using high-priced 50 low volatile coal. In the manufacture of coke, difficulties are encountered if high volatile coal is treated according to known coking processes, among which difficulties may be mentioned the fact that the coke fingers are small and are not marketable for many purposes.

A further object of the present invention is to provide an improved process whereby the percentage of cell structure of the coke may be controlled whereby to produce desired characteristics. It has been discovered that the thickness as well as the viscosity of the material in the coking zone varies rather closely in accordance with the coking qualities of the coal. Coal having a high coking power will present in the Knowles type of oven during the coking process a thicker and more viscous material in the coking zone than will a coal of low coking power. It is a further object, therefore, of the present invention to provide a process of coking by which the coking power of the charge may be modified to change the viscosity and thickness of the material in the coking zone and to produce any desired variation, within limits, with respect to the total volume of cells and the size of said cells in the resulting coke.

Further objects will appear as the description proceeds.

Figure 1 of the drawing is a more or less diagrammatic representation of the action within a Knowles type of oven operated according to the present invention; and

Figure 2 is a diagrammatic view illustrating a cycle of operation according to the present invention.

In said diagram the horizontal oven floor is indicated by the numeral 1 and the roof thereof is indicated by the numeral 2. Side walls are indicated by the numerals 3—3. The oven is shallow relative to its width and length. The horizontal floor 1 is heated by means of gases passing through flues 4—4 below said floor. Coal or equivalent material is disposed upon said floor 1. Means (not shown) will be provided for charging coal into the oven chamber, other means, such as the uptake 4a, will be provided for withdrawing gases and vapors, and means will also be provided for sealing the ends of the chamber. The oven will be so constructed that a charge of material, after having been treated, may be pushed out of the coking chamber. Figure 1 of the drawing represents conditions when a particular heat treatment has been completed and the charge is ready to be pushed out of the coking chamber. Under these conditions the charge within the coking chamber will be in three rather distinct layers, indicated by the numerals 5, 6 and 7. The lowermost layer 5 according to the present invention will be coke, the various fingers of which are indicated by the numerals 5a—5a. Above the layer 5 of coke is a layer of plastic material 6, which layer is always at approximately the softening temperature of the coal being treated. This plastic layer 6 will in service be a tarry mass in which the coal has become liquefied. Above the layer 6 is a layer 7 of coal in unfused condition. The coal in layer 7 has a temperature always below the softening temperature of the coal. In service a certain amount of hot gases from the coke zone 5 will pass laterally to the walls and upwardly into the chamber above the layer 7. Under these conditions the topmost portion of the layer 7 may be in swollen condition, but in service the coal in the layer 7, even at the topmost portion thereof, will not be fused. An explanation of this phenomenon which occurs to applicant is that the gases passing upwardly from the plastic layer 6 become cooled in passing through the layer 7 and prevent the fusing of even the uppermost portion of said layer 7. Moreover, the hot gases passing

upwardly along the side walls will tend to pass off through the uptake 4a, whereby said layer 7 will be protected against temperatures above the fusing temperature of the coal in said layer 7.

The heat treatment according to the present invention is carried on from the bottom of the charge toward the top, where the upper part of the charge, that is—in the layer 7, is considerably devolatilized but is not changed in its physical form. The only change in the layer 7 is the driving out of moisture and part of the volatile matter, that is—those volatiles which come off at temperatures below the softening temperature of the coal. According to the present invention there is no fusing of the upper part of the charge, inasmuch as the temperatures at that region are below the fusing temperature of the coal. As indicated above, the temperature conditions in the upper part of the charge should be maintained at a value below the softening temperature thereof, to the end that the physical form of the coal in the upper part of the charge is not materially changed. When the material in the lower part of the charge, that is—in the layer 5, has been coked and while the material in the upper portion of the charge, that is—in the layer 7, is in its partially devolatilized unfused condition, the charge is removed from the oven.

The manner in which the material may be treated will depend largely upon the individual practical conditions confronting the operator. If preferred, the charge, after being cooled, may be screened to remove the largely devolatilized pieces of soft coke resulting from the breaking up of the layer 6 and to remove the partially devolatilized coal. According to the step referred to, these pieces of coke and partially devolatilized coal are preferably crushed, although crushing is not essential. According to a process at present preferred, the pieces of coke and partially devolatilized coal are crushed to a size which will pass through a ten mesh screen. This material, preferably in crushed condition, is intimately mixed with the coal in the next batch to be treated. It will be understood that the intimacy of the mixture may be promoted by grinding the coal to relatively small size. By varying the proportions of the soft coke and partially devolatilized coal with respect to the coal to be treated, it is possible to produce coke of the physical characteristics usually desired.

Figure 2 indicates diagrammatically the cycle of operation. After the treatment in the Knowles type of oven as above described, the charge is pushed out of the oven and the partially devolatilized coal and soft coke are separated from the commercial or hard coke. The partially devolatilized coal and soft coke are then mixed with fresh coal for the next batch.

In practice in the manufacture of coke, the run-of-oven product is usually crushed and sized as required by market conditions. The smaller pieces, for example that which passes through a  $\frac{1}{2}$  to  $\frac{3}{4}$  inch screen, is commonly called braize. This braize has no particular function according to the present invention, but for practical purposes may be included along with the soft, mildly coherent coke and the partially devolatilized coal. The broken pieces of hard coke, which form only a small percentage of the braize, have little or no binding power, but the soft, mildly coherent coke and the partially devolatilized coal have a surface affinity for tar vapors and melting bitumen, and the mixture with raw coal produces a more thoroughly melted and cemented coke.

than can be obtained from a mixture of high temperature braize and coal.

If preferred, the charge which has been removed from the oven may be treated as follows:

- 5 The upper layer 1 of said partially devolatilized coal is separated from the fused, more or less coherent layer 6, which layer is composed of soft coke. The soft coke comprising said layer 6 may be utilized along with the hard coke resulting 10 from the layer 5. With some types of coal the layer 6 of soft, mildly coherent coke will screen off with the partially devolatilized coal in layer 1. With other types of coal, this layer 6 will screen off with the coke in layer 5. The pieces 15 of partially devolatilized coal resulting from the layer 1 are in condition to be mixed with a succeeding batch to produce coke of the desired characteristics. Expressed in other language, the partially devolatilized coal which has been produced 20 from high volatile coal now presents many of the desirable characteristics of mined low volatile coal. The pieces of partially devolatilized coal are preferably crushed, although crushing is not essential. This partially devolatilized coal, preferably in crushed condition, is intimately mixed with fresh coal in the next 25 batch to be treated. It will be understood that the intimacy of the mixture may be promoted by grinding the coal to relatively small size. By 30 varying the proportions of the partially devolatilized coal with respect to the raw coal in a batch, it is possible to produce coke of the physical characteristics usually desired. The partially devolatilized coal has a surface affinity for 35 tar vapors and melting bitumen, and the mixture with raw coal produces a more thoroughly melted and cemented coke than can be obtained from a mixture of high temperature braize and coal, or than can be obtained from high volatile coal itself.

According to the present invention the partially devolatilized coal of the desired quality is produced in one operation at the same time and in the same process at which the high temperature coke is made. The addition of, for example, a two-inch extra height of coal on top of the normal charge of coal improves the heat economy of the process, because these two inches of material, when heated to the lower temperature as contemplated by the present invention, radiate less heat from the charge, and by the insulating effect thereof assist the coke below to reach the high temperature desired. It may be stated at this point that no difficulties arise from the presence of the low temperature partially devolatilized coal on top of the high temperature coke, but, on the contrary, the addition of the extra height of coal on top of the normal charge will exert a pressure upon the lower coal and thus help to reduce its porosity, and thus make it suitable for certain metallurgical processes.

According to the present invention the special partially devolatilized coal referred to may be added to the raw coal in relatively large percentages, giving in the case of certain coals a very high grade, high temperature coke.

The partially devolatilized coal contemplated in the present invention has a different function than braize would have, in that the material contemplated herein unites homogeneously with the raw coal in the same manner as a low volatile coal, which costs more money in many localities. With braize the uniting of said braize is not with the raw coal but with the coke. The 75 result of this last mentioned union is a poorer

bond than is the case with the uniting of the two coals. It may be noted that in order to produce a desirable coke which will stand handling without undue breakage it is necessary to use in the manufacture of said coke a low volatile coal to the extent of 15 to 25 per cent of the mixture. The present invention makes it possible to utilize a high volatile coal, and, by treating as described, to obtain a sufficiently low volatile coal to accomplish the purpose.

It is intended to cover all modifications of the present invention that fall within the scope of the appended claims.

What is claimed is—

1. The cyclic process of producing coke which consists in providing a bed of high volatile, cokable coal shallow relative to its width and length, applying heat thereto below said bed to coke the lower portion of said bed, stopping the coking process at a point which will produce a predetermined amount of partially devolatilized coal and mildly coherent soft coke at the top of the charge, which partially devolatilized coal has the moisture driven therefrom and those volatiles removed which come off below the softening temperature of said high volatile, cokable coal, separating this devolatilized coal and soft coke from the hard coke produced below it, mixing said devolatilized coal and soft coke with a succeeding charge of coal, and repeating the 30 coking process referred to.

2. The method of preparing coke which consists in intimately mixing with high volatile, cokable coal a predetermined portion of partially devolatilized coal and mildly coherent soft coke, 35 heating from below a shallow bed of said mixture to coke the lower portion of said bed and stopping the heating process at a point which will produce a predetermined amount of partially devolatilized coal and mildly coherent soft coke on top of said bed, which partially devolatilized coal has the moisture driven therefrom and those volatiles removed which come off below the softening temperature of said high volatile, cokable coal and separating out the desired constituents resulting 45 from said operation.

3. The process of producing coke of desired physical characteristics with respect to size and total volume of pores which consists in mixing soft coke and largely devolatilized coal with a charge of high volatile, cokable coal, heating from below a shallow bed of said mixture to coke the lower portion of said bed, and stopping the heating process at a point which will produce a predetermined amount of partially devolatilized coal and mildly coherent soft coke on top of said bed, which partially devolatilized coal has the moisture driven therefrom and those volatiles removed which come off below the softening temperature of said high volatile, cokable coal.

4. The cyclic process of producing coke of desired physical characteristics with respect to size and total volume of pores which consists in mixing soft coke and largely devolatilized coal with a charge of high volatile, cokable coal, heating 65 from below a shallow bed of said mixture to coke the lower portion of said bed, stopping the heating process at a point which will produce a predetermined amount of partially devolatilized coal and mildly coherent soft coke on top of said bed, which partially devolatilized coal has the moisture driven therefrom and those volatiles removed which come off below the softening temperature of said high volatile, cokable coal, removing said devolatilized coal and soft coke from 75

said charge, and mixing said devolatilized coal and soft coke with coal for a succeeding coking charge.

5. The cyclic process of producing coke which 5  
5 consists in providing a bed of high volatile, cokable coal shallow relative to its width, applying heat thereto below said bed to coke the lower portion of said bed, stopping the coking process at a point below that which will fuse the top 10  
10 portion of said bed but which will drive off the moisture from and cause a partial devolatilization of the coal in the upper portion of said bed, removing the resulting devolatilized coal, mixing 15  
15 said devolatilized coal with a succeeding charge of high volatile, combustible coal, and repeating the coking process referred to.

6. The method of producing a partially devolatilized coal suitable for coking purposes which 15  
20 consists in providing a bed of coal shallow relative to its width, applying heat thereto below said bed, stopping said heating process at a point at which the lower portion of said bed is coked and at which the moisture and part of the volatiles are driven off from the upper portion 25  
25 of said bed but below a point which will cause fusion of the coal in the upper portion of said bed, and separating the partially devolatilized coal from the remainder of the charge.

7. The process of producing coke of desired 30  
30 physical characteristics with respect to size and total volume of pores which consists in mixing largely devolatilized coal in unfused condition with a charge of high, volatile, cokable coal and heating from below a shallow bed of said mixture, limiting the time of said heating step so 35  
35 that only the lower portion of said bed is coked and the upper portion of said bed has its moisture removed and is in partially devolatilized but unfused condition.

8. The cyclic process of producing coke of desired physical characteristics with respect to 40  
40

size and total volume of pores which consists in mixing largely devolatilized coal in unfused condition with a charge of high volatile, cokable coal, heating from below a shallow bed of said mixture to coke the lower portion of said bed, stopping the heating process at a point which will produce a predetermined amount of partially devolatilized coal in unfused condition, which coal has its moisture and part of its volatiles driven therefrom, removing said devolatilized coal from said charge, and mixing said devolatilized coal with raw coal for a succeeding coking charge.

9. The method of producing a physically strong coke in a cyclic operation which consists in coking a mixture of high volatile, cokable coal and partially devolatilized material such as produced in a later step of the operation, heating this mixture in a flat layer from below, carrying said heating operation to a point where a hard, physically strong coke and a layer of partially devolatilized coal are produced which partially devolatilized coal has the moisture driven therefrom and those volatiles removed which come off below the softening temperature of said high volatile, cokable coal, separating the coke from the partially devolatilized coal, and returning the partially devolatilized material to the first step of the operation.

10. The method of producing a physically strong coke which consists in coking a mixture of high volatile, cokable coal and relatively low volatile coal, heating this mixture in a flat layer from below, carrying said heating operation to a point where a hard, physically strong coke and a layer of partially devolatilized coal are produced, which partially devolatilized coal has the moisture driven therefrom and those volatiles removed which come off below the softening temperature of said high volatile, cokable coal.

MAURICE D. CURRAN.